

Nov. 6, 1934.

H. SPRUNG

1,980,011

METHOD FOR THE PRODUCTION OF MAGNETIC STRIPS OR TAPES

Filed Aug. 11, 1933



INVENTOR  
H. SPRUNG  
BY *Harry E. Durham*  
ATTORNEY

## UNITED STATES PATENT OFFICE

1,980,011

METHOD FOR THE PRODUCTION OF  
MAGNETIC STRIPS OR TAPES

Helmut Sprung, Berlin-Oberschoneweide, Germany, assignor to General Electric Company, Schenectady, N. Y., a corporation of New York

Application August 11, 1933, Serial No. 684,771  
In Germany August 16, 1932

6 Claims. (Cl. 175—21)

It has previously been proposed to produce sheet metal, wire, and strip cores and Krarup windings which are made of a ferromagnetic material which after any desired saturation with 5 direct current field, has an instability of less than 5% with an initial permeability of  $\mu_0=25$  and more. In the production of strip cores it has been found that when the strip is simply wound up, the elastic stresses set up in it, lead to an appreciable 10 deterioration of the magnetic properties, particularly the hysteresis. On this account it has been proposed in the case of strip cores to obtain the requisite bending by plastic deformation either by bending the strip at regular intervals or by 15 first winding the strip on a very much thinner mandrel and subsequently allowing it to expand to the desired diameter. The first process is accompanied by the disadvantage that the core no longer possesses a circular shape and can therefore 20 only be wound with an uneconomical utilization of the available space; the second process possesses the disadvantage that the core after expanding can no longer be wound so tightly.

The object of the invention is to provide a 25 process for the production of strip cores in which these disadvantages are eliminated by plastically deforming the strip of ferromagnetic material a number of times in different directions before it is wound into a core so that it loses its springiness to an appreciable extent and it is then given 30 a final change of shape such that it does not exhibit any further elastic tension after being wound up. For this purpose the plastic deformation and winding may advantageously be carried out in one working process. The repeated 35 plastic deformation may be done in various ways. One process which has been found particularly suitable is that in which the strip is drawn between two rows of rollers which are set with respect to one another in such a way that the rollers 40 in one row stand opposite the gaps in the other row and engage in these gaps. The diameter of the rollers in one row is preferably selected somewhat greater than the diameter of the rollers 45 in the other row.

A diagram of one apparatus suitable for the production of strip cores according to the invention is illustrated in the drawing by way of example.

50 In the drawing the strip 1 is wound into a core 3 on the mandrel 2. The mandrel may be driven in any desired manner, for example, by means of gear wheels 4 and 5. Before being wound up, the strip is plastically deformed a number of 55 times in opposite directions according to the in-

vention by drawing it between the rollers 6 and 7 which may consist of steel for example. The rollers are arranged in such a way that the rollers 7, the diameters of which are the smaller, are always opposite the gaps in the rollers 6. The 60 distance apart of the two rows of rollers may be altered by means of the pressure screw 8, according to the nature and composition of the material employed. The smaller the distance between the two rows of rollers is, or the more the rollers having the smaller diameter project into the gaps between the rollers having the larger diameter, the greater will be the plastic deformation. On leaving the rollers the strip will have a permanent bend on the side of the smaller rollers. This 65 bend must be of such size that the strip on being wound up will possess little or no elastic tension. The size of the bend will depend upon the diameter of the rollers and their mutual position with respect to one another and also upon the tensile 70 stress during the drawing operation, as the bend may be partially neutralized by the tensile stress. In accordance with the diameter of the core to be wound, therefore, the separate factors must be 75 adjusted in such a way that the bend has the requisite size. Furthermore, precautions must, of course, be taken that the strip receives its permanent bend in the direction in which it is subsequently to be bent as a core.

The above described method of production 80 possesses the further advantage that any rough edge or ridge formed by cutting the strips is pressed flat by the rollers so that a special flattening process is rendered unnecessary.

The insulation of the strip core is carried out 85 in a known manner. Since the core will have no further spring expansion after being wound, it is possible to allow a thin paper strip to run in with it, very little danger existing of the paper strip tearing, which was often the case in the hitherto customary process. Moreover, insulation 90 may also be applied by impregnating the strip before or after winding in any liquid or easily readily flowing insulating medium, such as lacquer or like insulating mediums, and further in isinglass or similar materials and generally in all insulating mediums which are employed for solid cores.

What is claimed is:

1. Process for the production of strip cores of magnetic material to be employed in cold worked form, characterized in that the strip for winding the cores is plastically deformed a number of times in alternate directions before being wound up, so that it loses its spring power to an appre-

- ciable extent, and that it is at the same time given a final change of form of such a kind that it no longer exhibits any elastic tension after being wound up.
5. 2. Process according to claim 1, characterized in that the plastic deformation is carried out in one working process with the winding.
3. Process according to claim 1, characterized in that the change of shape which is given to 10 the strip in the direction of the last plastic deformation is partially removed again by winding in a corresponding direction to relieve the tensile stress.
4. Process according to claim 1, characterized by that for purposes of insulation a thin paper strip is wound up parallel with the strip itself.
5. Process according to claim 1, characterized in that the strip is impregnated in a liquid or 80 readily flowing insulating medium before or after winding.
6. Process according to claim 1, characterized in that the strip is insulated by chemical treatment of the surface. 85

HELMUT SPRUNG.

15

90

20

95

25

100

30

105

35

110

40

115

45

120

50

125

55

130

60

135

65

140

70

145

75

150